# EUROPEAN PATENT SPECIFICATION

(11) **EP 1 420 041 B1**
(45) Date of publication and mention of the grant of the patent: **14.04.2010**
(21) Application number: 03078703.0
(22) Date of filing: 18.11.2003
(51) Int. Cl.: C08J 7/04, E04D 5/10, E04D 12/00

(54) **A flexible sheet material**
Flexibles Folienmaterial
Matériau en feuille souple

(30) Priority: 18.11.2002 DK 200201772
(43) Date of publication of application: 19.05.2004
(73) Proprietor: ICOPAL A/S, 2730 Herlev (DK)
(72) Inventor: Harder, Sven, 2625 Vallensbaek (DK); Jensen, Eirik Sandberg, 40000 Roskilde (DK)
(74) Representative: Plougmann & Vingtoft A/S

(56) References cited:
- DE-U- 20 019 212

## Description

### Technical field

The present invention relates to a fire resistant flexible sheet material with a high water vapour diffusion resistance and a low gross calorific potential. The flexible sheet material may advantageously be used as a water vapour barrier in roof constructions.

### Background of the invention

When the heat insulation is placed on the outside of the load-bearing construction as in for example steel deck constructions, the heat insulation is placed between two water impermeable membranes, i.e. the water vapour barrier and the roofing. This type of roof construction imposes requirements on the water vapour barrier used. To ensure that moisture is not accumulated in the insulation layer, the water vapour diffusion resistance of the water vapour barrier should be high, due to a high water vapour diffusion resistance of the roofing. The building code imposes requirements on the water vapour barrier with regard to the gross calorific potential which, as a consequence of fire classification of construction products and building elements, must be low.

Traditionally, a laminate including an aluminium foil has been used to obtain a water vapour barrier with a high water vapour diffusion resistance. However, the aluminium foil requires corrosion protection, e.g. with polyethylene, in order to prevent corrosion thereof, when the water vapour barrier is placed in a humid environment, such as in a roof construction or in a construction in swimming baths. A corrosion protection in the form of e.g. polyethylene will add to the gross calorific potential of the water vapour barrier and impede the fulfilment of the requirements of the building code. Moreover, if the flames used for attaching the roofing felt accidentally hit the laminate including an aluminium foil, e.g. along a skylight or ventilator cowl, the aluminium will act as a fire spreader and the fire may spread down through the roof construction. The problem cannot be solved by adding a large amount of fire retardant to the laminate due to the fact, that the second film of the laminate, i.e. the plastic film, cannot adhere to the aluminium foil, when using a large amount of fire retardant.

DE 200 19 212 U discloses a barrier laminate comprising an aluminum foil acting as a water vapour membrane, which is coated on one side with a layer of plastic such as, for example polyethylene terephthalate, while on the other side it is coated with a non combustible lacquer for protection against corrosion and for improving adhesion between aluminum and a bitumen layer. Its use in roofing and its method of making are as well described therein.

WO 00 37751 discloses a water vapour multi layer barrier film, that comprises a first, water impervious membrane having a plurality of first through openings defined therein, and a second, water impervious membrane which is arranged opposite to the first membrane; the whole film exhibits a "heating value" not exceeding 4 MJ/m·2· One of the membranes, or an additional layer of the barrier film can be made of polyamide resin in order to improve fire retardant properties. Usually, the water vapour diffusion resistance of the first membrane, which is said to be substantially impervious to water vapour, should be equivalent to 10-100 m air column at any relative humidity of air in contact therewith, but the water vapour diffusion resistance may also be equivalent to 2000 m air column or even higher depending on the chosen material.

### Summary of the invention

It is an object of the present invention to provide a flexible sheet material that is applicable as a water vapour barrier and, furthermore, fulfils the conflicting requirements mentioned above, i.e. a flexible sheet material with a high water vapour diffusion resistance and a low gross calorific potential.

According to a preferred embodiment of the present invention, there is provided a flexible sheet material comprising a first film or membrane of a plastic material having a thickness of less than 50 µm, wherein said film or membrane has a substantially non-combustible coating so as to obtain a water vapour diffusion resistance of the sheet material exceeding 45 m air column and a gross calorific potential not exceeding 4 MJ/m², and further comprising intumescent graphite as a fire retardant within or adjacent to said first film or membrane.

The gross calorific potential is defined as the calorific value of a material, when the combustion is complete and any produced water is entirely condensed, and the calorific value is defined as the thermal energy produced by combustion of unit of mass of a given substance.

In order to reduce the gross calorific potential of the flexible sheet material, the thickness of the film or membrane is reduced compared to traditional water vapour barriers with a high water vapour diffusion resistance. To obtain a high water vapour diffusion resistance, the film or membrane is coated with a substantially non-combustible coating.

The thickness of the first film or membrane may be less than 40 µm, such as less than 30 µm or less than 25 µm.

Furthermore, the film or membrane may in one embodiment be coated with a substantially non-combustible coating so as to obtain a water vapour diffusion resistance of the sheet material exceeding 60 m air column.

A second film or membrane may be laminated to the first film or membrane. Laminating the second film or membrane at the coated side of the first film or membrane, the second film or membrane may be used as a protection for the coating of the first film or membrane, whereby the sheet material may be used in e.g. a harsh environment.

The flexible sheet material further comprises a fire retardant. The fire retardant may be arranged in any position within or adjacent to the first film or membrane. Thus, it may be arranged between the first and second films or membranes, and in a preferred embodiment the fire retardant may be incorporated in an adhesive layer arranged between the first and second films or membranes. The adhesive layer may comprise urethane, epoxy or other glue, an adhesive web or film, or others.

The fire retardant used in the flexible sheet material according to the invention is intumescent graphite, which may expand to a volume being up to 100 times the initial volume.

The second film or membrane may be coated with a substantially non-combustible coating in order to obtain a flexible sheet material comprising two films or membranes being coated with a substantially non-combustible coating, whereby the thickness of each of the films may be reduced without reducing the water vapour diffusion resistance of the sheet material.

Furthermore or alternatively, the second film or membrane may comprise a porous fibrous material, such as felt with a low calorific value, e.g. Nylon felt or glass felt. By the use of a porous fibrous material, the second film or membrane may serve as a sound absorber and/or as physical protection of the flexible sheet material.

The first film or membrane may comprise a layer of a plastic material. Furthermore, the second film or membrane may also comprise a layer of a plastic material. As an example, the plastic material may be polyethylene terephthalate (PETP), polyethylene naphthalate (PEN), or copolymers thereof, oriented polypropylene (OPP), polyethylene (PE), oriented polyamide (OPA), Cyclic Olefinic Copolymers (COC) or Aclar, Aclar being a flexible thermoplastic made of fluorinated-chlorinated resins. Other plastic materials may also be used.

An example of an Aclar-film is Aclar CxTM8A (33 µm), which is a heat-sealable polychlorotrifluoroethylene (PCTFE) homopolymer film co-extrusion. The structure consists of an 8 µm Aclar film layer laminated to a 25 µm layer of polyethylene (PE).

The films or membranes may be coated with a substantially non-combustible coating, such as silicon oxide, aluminium oxide, aluminium or polyvinylidenechloride. The films or membranes may be coated more than once using one or more of the coatings in combination, whereby a synergy effect may be achieved in that one film or membrane coated twice may be used instead of using a laminate of two films or membranes each coated once. An example of a combination of coatings is a PVdC-coating (polyvinylidenechloride) followed by an aluminium coating. Another example is an EVOH-coating (ethylene vinyl alcohol) followed by an aluminium coating. Other combinations may also be used.

The coating using silicon oxide (SiOₓ), aluminium oxide or aluminium may be performed under low pressure and high temperature, such as a plasma deposition coating. By the use of plasma deposition coating a thin coating with an even surface structure may be obtained. Condensation or spray coating may also be used. The coating using polyvinylidenechloride may be performed as a standard coating process using gravure rollers and drying tunnel. However, other coating processes may also be used.

In order to increase the strength of the sheet material, it may further comprise reinforcing means. The reinforcing means may be arranged in any position adjacent to the first film or membrane. Thus, it may be arranged between the first and second films or membranes, and in a preferred embodiment, the reinforcing means may be incorporated in an adhesive layer arranged between the first and second films or membranes. The reinforcing means may comprise a netting. As an example, the reinforcing means may be made of glass, polypropylene, polyester or polyethylene.

In another preferred embodiment of the present invention, the flexible sheet material may have a gross calorific potential not exceeding 2 MJ/m².

In a third preferred embodiment of the present invention, the flexible sheet material may have a gross calorific potential not exceeding 1.4 MJ/m², and/or a water vapour diffusion resistance exceeding 90 m air column.

According to other preferred embodiments of the present invention a flexible sheet material is used as a water vapour barrier or an underroof for buildings. The flexible sheet material comprise a first film or membrane of a plastic material having a thickness of less than 50 µm, and this first film or membrane has a substantially non-combustible coating so as to obtain a water vapour diffusion resistance of the flexible sheet material exceeding 45 m air column and a gross calorific potential of the flexible sheet material not exceeding 4 MJ/m², and intumescent graphite is present as a fire retardant within or adjacent to said first film or membrane.

Any of the features of the flexible sheet material according to the invention may be used in combination with the flexible sheet material used as a water vapour barrier or as an underroof for buildings.

According to European Standard EN 13501-1, a non-homogeneous product is a product composed of one or more components which may be substantial or non-substantial. A non-substantial component is a material which does not constitute a significant part of a non-homogeneous product. Furthermore, a layer with a mass/unit area of less than 1.0 kg/m² and a thickness of less than 1.0 mm is considered to be a non-substantial component. An internal non-substantial component is defined as a non-substantial component covered on both sides by at least one substantial component, whereas an external non-substantial component is not covered at one side of a substantial component. As a consequence of these definitions, a water vapour barrier may be classified as an external non-substantial component of a non-homogeneous product.

According to the requirements of EN 13501-1, the gross calorific potential of a water vapour barrier, i.e. an external non-substantial component of a non-homogeneous product should not exceed 2 MJ/m², when belonging to class A1. Furthermore, the gross calorific potential of a water vapour barrier, i.e. an external non-substantial component of a non-homogeneous product should not exceed 4 MJ/m², when belonging to class A2. Class A1 and A2 are the two highest classes in the classification of reaction to fire performance for construction products being tested in accordance with the Standard, class A1 being higher than A2 as the requirements of A1 are more strict than the requirements of A2.

### Brief description of the drawings

Embodiments of a flexible sheet material according to the present invention are for illustration of the invention described below with reference to the accompanying drawings of which
Figs. 1-4 show sectional views of four different embodiments of a flexible sheet material.

### Detailed description of the drawings

Fig. 1 is a sectional view of a first embodiment of a flexible sheet material according to the invention. The flexible sheet material comprises upper and lower layers, 10 and 11, respectively, of coated films of polyethylene terephthalate each having a thickness of 12 µm. The polyethylene terephthalate films are coated with silicon oxide. The upper layer 10 is laminated to the lower layer 11 by means of an intermediate adhesive layer 12, such as urethane glue of approximately 2 µm, having a fire retardant, such as intumescent graphite, incorporated therein. The gross calorific value of this flexible sheet material is 0.8 MJ/m², and the water vapour diffusion resistance is 180 m air column.
Fig. 2 is a sectional view of a second embodiment of a flexible sheet material according to the invention. The second embodiment also comprises upper and lower layers, 10 and 11, of coated films of polyethylene terephthalate each having a thickness of 12 µm. Also these layers are laminated together by an adhesive layer 12, such as urethane glue of approximately 2 µm, having a fire retardant, such as intumescent graphite, incorporated therein. Furthermore, a glass netting 13 is incorporated in the adhesive layer 12 in order to increase the strength of the flexible sheet material. The gross calorific value of this flexible sheet material is 1.0 MJ/m², and the water vapour diffusion resistance is 150 m air column.
Fig. 3 illustrates a sectional view of a third embodiment of a flexible sheet material according to the invention. The flexible sheet material illustrated in Fig. 3 comprises an upper layer 10 formed by a coated film of polyethylene terephthalate having a thickness of 12 µm laminated to an intermediate film 14 of polyethylene with a thickness of 30 µm. An adhesive layer 12, such as urethane glue of approximately 2 µm, having a fire retardant, such as intumescent graphite, incorporated therein is arranged between the upper layer 10 and the intermediate layer 14. A lower lever 15 of glass felt with a thickness grammage of 50 gr/m² is laminated to the intermediate film 14 of polyethylene. The gross calorific value of this flexible sheet material is 2.2 MJ/m², and the water vapour diffusion resistance is 98 m air column.
Fig. 4 illustrates a sectional view of a flexible sheet material that is not according to the invention. The flexible sheet material of Fig. 4 comprises an upper layer 10 of coated polyethylene terephthalate having a thickness of 12 µm laminated to a lower layer 11 of co-extruded oriented polypropylene having a thickness of 18 µm by an intermediate adhesive layer 12 in the form of urethane glue of approximately 2 µm. The gross calorific value of this flexible sheet material is 1.8 MJ/m², and the water vapour diffusion resistance is 82 m air column.

## Claims

1. A flexible sheet material comprising a first film or membrane of a plastic material and having a thickness of less than 50 µm, wherein said film or membrane has a substantially non-combustible coating so as to obtain a water vapour diffusion resistance of said sheet material exceeding 45 m air column and a gross calorific potential of said sheet material not exceeding 4 MJ/m² and further comprising intumescent graphite as a fire retardant within or adjacent to said first film or membrane.

2. A flexible sheet material according to claim 1, wherein the thickness of said first film or membrane is less than 30 µm.

3. A flexible sheet material according to claim 1 or 2, wherein said film or membrane has a substantially non-combustible coating so as to obtain a water vapour diffusion resistance of said sheet material exceeding 60 m air column.

4. A flexible sheet material according to any of the preceding claims, further comprising a second film or membrane laminated to said first film or membrane.

5. A flexible sheet material according to claim 4, wherein the fire retardant is incorporated in an adhesive layer arranged between said first and second films or membranes.

6. A flexible sheet material according to any of claims 4 or 5, wherein the second film or membrane is coated with a substantially non-combustible coating.

7. A flexible sheet material according to any of claims 4-6, wherein the second film or membrane comprises a porous fibrous material.

8. A flexible sheet material according to claim 7, wherein the second film or membrane comprises Nylon felt or glass felt.

9. A flexible sheet material according to any of claims 4-8, wherein the second film or membrane comprises a layer of a plastic material.

10. A flexible sheet material according to any preceding claim, wherein the plastic material is selected from the group consisting of polyethylene terephthalate (PETP), polyethylene naphthalate (PEN), or copolymers thereof, oriented polypropylene (OPP), polyethylene (PE), oriented polyamide (OPA), Aclar and Cyclic Olefinic Copolymers (COC).

11. A flexible sheet material according to any of the preceding claims, wherein the coating of said first and/or second film or membrane comprises at least one material selected from the group consisting of silicon oxide, aluminium oxide, aluminium and polyvinylidenechloride.

12. A flexible sheet material according to any of the preceding claims and further comprising reinforcing means for increasing the strength of the sheet material.

13. A flexible sheet material according to claim 12, wherein the reinforcing means comprises a netting.

14. A flexible sheet material according to claim 12 or 13, wherein the reinforcing means is made of a material selected from the group consisting of glass, polypropylene, polyester, and polyethylene.

15. A flexible sheet material according any of the preceding claims, and having a gross calorific potential not exceeding 2 MJ/m².

16. A flexible sheet material according to claim 15, wherein the gross calorific potential does not exceed 1.4 MJ/m².

17. A flexible sheet material according any of the preceding claims, wherein the water vapour diffusion resistance exceeds 90 m air column.

18. Use of a flexible sheet material as a water vapour barrier or underroof for buildings, said flexible sheet material comprising a first film or membrane of a plastic material and having a thickness of less than 50 µm, wherein said film or membrane has a substantially non-combustible coating so as to obtain a water vapour diffusion resistance of said sheet material exceeding 45 m air column and a gross calorific potential of said sheet material not exceeding 4 MJ/m² and further comprises intumescent graphite as a fire retardant within or adjacent to said first film or membrane.

## Patentansprüche

1. Biegsames Folienmaterial, umfassend einen ersten Film oder eine erste Membran aus einem Kunststoffmaterial und mit einer Dicke von weniger als 50 µm, wobei der Film oder die Membran eine im Wesentlichen nicht brennbare Beschichtung aufweist, um einen Wasserdampfdiffusionswiderstand des Folienmaterials von mehr als 45 m Luftsäule und einen Bruttoheizwert des Folienmaterials von nicht mehr als 4 MJ/m² zu erhalten, und weiterhin umfassend Blähgrafit als ein feuerhemmendes Mittel innerhalb des ersten Films oder der ersten Membran oder benachbart dazu.

2. Biegsames Folienmaterial nach Anspruch 1, wobei die Dicke des ersten Films oder der ersten Membran weniger als 30 µm beträgt.

3. Biegsames Folienmaterial nach Anspruch 1 oder 2, wobei der Film oder die Membran eine im Wesentlichen nicht brennbare Beschichtung aufweist, um einen Wasserdampfdiffusionswiderstand des Folienmaterials von mehr als 60 m Luftsäule zu erhalten.

4. Biegsames Folienmaterial nach einem der vorhergehenden Ansprüche, weiterhin umfassend einen zweiten Film oder eine zweite Membran, der bzw. die auf den ersten Film oder die erste Membran laminiert ist.

5. Biegsames Folienmaterial nach Anspruch 4, wobei das feuerhemmende Mittel in eine Klebschicht eingearbeitet ist, die zwischen dem ersten und zweiten Film oder der ersten und zweiten Membran angeordnet ist.

6. Biegsames Folienmaterial nach einem der Ansprüche 4 oder 5, wobei der zweite Film oder die zweite Membran mit einer im Wesentlichen nicht brennbaren Beschichtung beschichtet ist.

7. Biegsames Folienmaterial nach einem der Ansprüche 4-6, wobei der zweite Film oder die zweite Membran ein poröses Fasermaterial umfasst.

8. Biegsames Folienmaterial nach Anspruch 7, wobei der zweite Film oder die zweite Membran Nylonfilz oder Glasfilz umfasst.

9. Biegsames Folienmaterial nach einem der Ansprüche 4-8, wobei der zweite Film oder die zweite Membran eine Schicht aus einem Kunststoffmaterial umfasst.

10. Biegsames Folienmaterial nach einem der vorhergehenden Ansprüche, wobei das Kunststoffmaterial ausgewählt ist aus der Gruppe, bestehend aus Polyethylenterephthalat (PETP), Polyethylennaphthalat (PEN) oder Copolymeren davon, gerecktem Polypropylen (OPP), Polyethylen (PE), gerecktem Polyamid (OPA), Aclar und cyclischen olefinischen Copolymeren (COC).

11. Biegsames Folienmaterial nach einem der vorhergehenden Ansprüche, wobei die Beschichtung des ersten und/oder zweiten Films oder der ersten und/oder zweiten Membran mindestens ein Material umfasst, ausgewählt aus der Gruppe, bestehend aus Siliziumoxid, Aluminiumoxid, Aluminium und Polyvinylidenchlorid.

12. Biegsames Folienmaterial nach einem der vorhergehenden Ansprüche und weiterhin umfassend Verstärkungsmittel zur Erhöhung der Festigkeit des Folienmaterials.

13. Biegsames Folienmaterial nach Anspruch 12, wobei das Verstärkungsmittel ein Netzgewebe umfasst.

14. Biegsames Folienmaterial nach Anspruch 12 oder 13, wobei das Verstärkungsmittel aus einem Material hergestellt ist, ausgewählt aus der Gruppe, bestehend aus Glas, Polypropylen, Polyester und Polyethylen.

15. Biegsames Folienmaterial nach einem der vorhergehenden Ansprüche und mit einem Bruttoheizwert von nicht mehr als 2 MJ/m².

16. Biegsames Folienmaterial nach Anspruch 15, wobei der Bruttoheizwert nicht mehr als 1,4 MJ/m² beträgt.

17. Biegsames Folienmaterial nach einem der vorhergehenden Ansprüche, wobei der Wasserdampfdiffusionswiderstand mehr als 90 m Luftsäule beträgt.

18. Verwendung eines biegsamen Folienmaterials als Dampfsperre oder Unterdach für Gebäude, wobei das biegsame Folienmaterial einen ersten Film oder eine erste Membran aus einem Kunststoffmaterial und mit einer Dicke von weniger als 50 µm umfasst, wobei der Film oder die Membran eine im Wesentlichen nicht brennbare Beschichtung aufweist, um einen Wasserdampfdiffusionswiderstand des Folienmaterials von mehr als 45 m Luftsäule und einen Bruttoheizwert des Folienmaterials von nicht mehr als 4 MJ/m² zu erhalten, und weiterhin Blähgrafit als ein feuerhemmendes Mittel innerhalb des ersten Films oder der ersten Membran oder benachbart dazu umfasst.

## Revendications

1. Matériau en feuille souple comprenant un premier film ou membrane constitué d'une matière plastique et possédant une épaisseur inférieure à 50 µm, où ledit film ou membrane possède un revêtement essentiellement non combustible de manière à obtenir une résistance à la diffusion de vapeur d'eau dudit matériau en feuille supérieure à une colonne d'air de 45 m et un potentiel calorifique supérieur dudit matériau en feuille ne dépassant pas 4 MJ/m² et comprenant également du graphite intumescent comme retardateur de flamme à l'intérieur ou à côté dudit premier film ou membrane.

2. Matériau en feuille souple selon la revendication 1, où l'épaisseur dudit premier film ou membrane est inférieure à 30 µm.

3. Matériau en feuille souple selon la revendication 1 ou 2, où ledit film ou membrane possède un revêtement essentiellement non combustible de manière à obtenir une résistance à la diffusion de vapeur d'eau dudit matériau en feuille supérieure à une colonne d'air de 60 m.

4. Matériau en feuille souple selon l'une quelconque des revendications précédentes, comprenant également un deuxième film ou membrane stratifié sur ledit premier film ou membrane.

5. Matériau en feuille souple selon la revendication 4, où le retardateur de flamme est incorporé dans une couche adhésive disposée entre lesdits premier et deuxième films ou membranes.

6. Matériau en feuille souple selon l'une quelconque des revendications 4 ou 5, où le deuxième film ou membrane est recouvert d'un revêtement essentiellement non combustible.

7. Matériau en feuille souple selon l'une quelconque des revendications 4 à 6, où le deuxième film ou membrane comprend un matériau fibreux poreux.

8. Matériau en feuille souple selon la revendication 7, où le deuxième film ou membrane comprend un feutre de nylon ou un feutre de verre.

9. Matériau en feuille souple selon l'une quelconque des revendications 4 à 8, où le deuxième film ou membrane comprend une couche d'une matière plastique.

10. Matériau en feuille souple selon l'une quelconque des revendications précédentes, où la matière plastique est choisie dans le groupe consistant en polyéthylène téréphtalate (PETP), polyéthylène naphtalate (PEN), ou des copolymères de ceux-ci, polypropylène orienté (OPP), polyéthylène (PE), polyamide orienté (OPA), aclar et copolymères d'oléfines cycliques (COC).

11. Matériau en feuille souple selon l'une quelconque des revendications précédentes, où le revêtement desdits premier et/ou deuxième films ou membranes comprend au moins un matériau choisi dans le groupe consistant en oxyde de silicium, oxyde d'aluminium, aluminium et polychlorure de vinylidène.

12. Matériau en feuille souple selon l'une quelconque des revendications précédentes et comprenant également un moyen de renfort pour accroître la résistance du matériau en feuille.

13. Matériau en feuille souple selon la revendication 12, où le moyen de renfort comprend un filet.

14. Matériau en feuille souple selon la revendication 12 ou 13, où le moyen de renfort est constitué d'un matériau choisi dans le groupe consistant en verre, polypropylène, polyester et polyéthylène.

15. Matériau en feuille souple selon l'une quelconque des revendications précédentes, et possédant un potentiel calorifique supérieur ne dépassant pas 2 MJ/m².

16. Matériau en feuille souple selon la revendication 15, où le potentiel calorifique supérieur ne dépasse pas 1,4 MJ/m².

17. Matériau en feuille souple selon l'une quelconque des revendications précédentes, où la résistance à la diffusion de vapeur d'eau est supérieure à une colonne d'air de 90 m.

18. Utilisation d'un matériau en feuille souple comme pare-vapeur ou sous-toiture pour bâtiments, ledit matériau en feuille souple comprenant un premier film ou membrane constitué d'une matière plastique et possédant une épaisseur inférieure à 50 µm, où ledit film ou membrane possède un revêtement essentiellement non combustible de manière à obtenir une résistance à la diffusion de vapeur d'eau dudit matériau en feuille supérieure à une colonne d'air de 45 m et un potentiel calorifique supérieur dudit matériau en feuille ne dépassant pas 4 Mj/m² et comprenant également du graphite intumescent comme retardateur de flamme à l'intérieur ou à côté dudit premier film ou membrane.
